

Dec. 15, 1942.

H. M. NOEL

2,305,440

## BITUMEN OF HIGH SOFTENING POINT

Filed July 25, 1940



Henry M. Noel Inventor  
By J. C. Small Attorney

## UNITED STATES PATENT OFFICE

2,305,440

## BITUMEN OF HIGH SOFTENING POINT

Henry M. Noel, Summit, N. J., assignor to Standard Oil Development Company, a corporation of Delaware

Application July 25, 1940, Serial No. 347,353

11 Claims. (Cl. 196—74)

This invention relates to hard unoxidized bituminous materials, a process for preparing the same and more particularly it relates to an asphalt having a high softening point and a definite change in penetration with temperature.

It is especially suitable for the manufacture of molded asphalt products generally, such as electric storage battery boxes, and also in the manufacture of high grade baking enamels and Japans.

Asphalts to be used for electric storage box compounds, molded products and in the manufacture of paints and Japans must meet certain specifications defined by the manufacturers of such products. The manufacturers in drawing up their specifications considered a natural asphalt (gilsonite) as a standard and required the other asphalts to meet these specifications and if possible show improvement over the specifications adopted.

Accordingly, one of these standards for a constituent of battery box compound is that the asphalt should have a penetration between 14 and 18 at 150° F./100 grams/5 secs. as determined by test No. D5-25 of the American Society for Testing Materials (A. S. T. M.).

According to the same standard, the susceptibility factor should be between 27 and 35 as calculated by the following formula:

$$10 \times \left( \frac{\text{Penetration at } 150^{\circ} \text{ F./100 g./5 secs.}}{\text{Penetration at } 115^{\circ} \text{ F./200 g./5 secs.}} + \frac{\text{Penetration at } 185^{\circ} \text{ F./50 g./5 secs.}}{\text{Penetration at } 150^{\circ} \text{ F./100 g./5 secs.}} \right)$$

The softening point should be above about 260° F. as determined by the ring and ball method, test No. D36-26 of the A. S. T. M.

The ductility should be high, that is about 35 to 40 centimeters at 185° F. at the rate of 5 cm./min. as determined by test No. D113-35 of the A. S. T. M.

It is well known to crack a reduced crude oil to produce lighter hydrocarbons and a heavy fuel oil which is further distilled to produce a pitch bottom and a heavy gas oil. So far, however, attempts to produce an asphalt by these means which has the desired softening point and susceptibility relationship and other characteristics that natural gilsonite possesses have failed, for the reason that all the desired properties could not be secured at the same time.

It has now been found that it is only when the proper crude source, the proper cracking conditions and the proper distillation conditions

are all combined that the desired product is secured.

According to this invention paraffin-free asphaltic base crudes, especially those from the western part of Venezuela, are suitable for the production of asphalt having the desired softening point and susceptibility, and other characteristics. The crude coming from the Lagunillas field is particularly desirable. Unless this crude is treated under proper conditions however, the desired product will not be obtained. The asphaltic content must be cracked to a certain point but cracking beyond this point results in an asphalt which is not suitable for this purpose. The final distillation also must be carried out under conditions which will give the desired melting point without appreciable further cracking.

The optimum conditions will vary somewhat with varying feed stocks, which can best be determined by experiment whenever the quality of the starting material changes.

The present invention will be understood on reading the following description of a typical example and by referring to the drawing of a diagrammatical representation of one type of apparatus suitable for the herein described process.

A suitable oil, a paraffin-free asphaltic base crude, for example, Lagunillas crude, is passed through pipe 1 to a visbreaker coil 2 into a soaking drum 3 and through pipe 4 to fractionating tower 5. An overhead distillate is removed from the fractionating tower by means of outlet 6 and a side stream of gas oil from outlet 13. The cracking is regulated so that the bottoms consist of a fuel oil having a gravity viscosity relationship such as that of 8° A. P. I. gravity and a Furol viscosity of 1000 to 1400 seconds at 122° F. or of 9° A. P. I. and a Furol viscosity of 600 to 850 seconds at 122° F. Heavier or lighter bottoms having higher or lower viscosities, respectively, may be used although the preferred range is 8° to 9° A. P. I. gravity. Within this range the quantity of material to be finally distilled is the minimum commensurate with ease of handling a viscous solution. The fuel oil is removed through outlet 7, passed through heating coil 8, with or without the addition of steam through pipe 9 and flashed into a vacuum tower 10, where an absolute pressure of 25 to 100 mm. is maintained. Steam may be added to the coil 8 and to the bottom of the vacuum tower 10 by means of pipe 11 to aid in the distillation of the overhead distillate. It is preferred to add the major portion of the steam to the tower 10.

Steam is the total amount of 10 to 40 lbs. per barrel of feed stock is used. A bitumen of 320° to 420° F. softening point is removed from the bottom outlet 12.

The unoxidized bitumen removed from the bottom outlet of the tower has a specific gravity of 1.10 to 1.25 and is 0.5 to 1.5% insoluble in carbon disulfide. The maximum temperature used in the second heating coil 8 to heat the fuel oil is not above 800° F., preferably from 750° to 790° F. The conditions maintained are to avoid the formation of a carbon disulfide insoluble content in the bitumen.

Bitumen produced under these special conditions from Lagunillas crude of Venezuelan source is found to be most valuable in the preparation of plastics but minor portions of other similar type crudes may be added. The yields and equipment used may be varied, the latter may be batch as well as a continuous process.

*Example 1*

A Lagunillas and La Rosa mixture of crude having a gravity of 17.4° A. P. I. is cracked in the refinery in a so-called visbreaker without a soaker to obtain 58.4% of fuel oil of a gravity of 8.9° A. P. I. and 11.4% of a pressure distillate of 400° F. end point naphtha. The fuel oil is vacuum reduced to obtain a bitumen of 402° softening point and 1.266 specific gravity and 1.53% insoluble in carbon disulfide.

*Example 2*

A Lagunillas crude of about 17° A. P. I. gravity is subjected to a high temperature such as about 850° F. and a pressure not materially above 200 lbs. per sq. in., in a narrow confined stream in a coil and passed into a soaking drum. The cracked oil is then passed to a separator where an overhead distillate is recovered and bottoms of 8° A. P. I. gravity having a Furol viscosity of 1400 seconds at 122° F. is removed. This fuel oil is heated in a coil and passed to a separator using a flash zone pressure 86 mm. and steam to the extent of 19.25 pounds per barrel of feed stock added. The bottoms recovered is an asphalt having a softening point of 370° F. and a susceptibility of 33.

*Example 3*

A mixture of a major part of Lagunillas crude and a minor part of La Rosa bottoms having a gravity of 17.1° A. P. I. were cracked in refining equipment under such conditions as to give 14.4% of pressure distillate, 28.4% of gas oil and 57.2% of 9.1 A. P. I. gravity bottoms. The 9.1 A. P. I. gravity bottoms were distilled under vacuum to a 402° F. softening point, 1.266 specific gravity, 1.53% insoluble in carbon disulfide, susceptibility of 27 and satisfactory ductility.

The bitumens obtained by this process have the desired susceptibility factor of 27 to 35 calculated by the above formula. The advantage of a bitumen prepared from the above stocks, by the above described particular preliminary cracking conditions and subsequent distilling conditions is that of having a higher softening point asphalt than any unoxidized bitumen prepared commercially from petroleum oils while likewise having low percent insoluble in carbon disulfide, the desired susceptibility factor, ductility and the other special properties characteristic of natural gilsonite.

A further improved characteristic of this asphalt is that a higher softening point than that of gilsonite may be obtained. The proportion of bituminous material entering in the preparation of battery boxes is about 3.5%, the other material being inert inorganic fillers, etc.

I claim:

1. A hard unoxidized bituminous material adapted for use in a storage battery compound derived from cracked and vacuum distilled paraffin-free asphaltic base petroleum crude oil having a susceptibility factor between 27 and 35, and a softening point between 320° F. and 420° F. and a content of material insoluble in carbon disulfide less than 1.5%.

10 2. A hard bituminous material adapted for use in a storage battery compound derived from a cracked and vacuum distilled West Venezuela petroleum crude having a susceptibility factor between 27 and 35 and a softening point between 320° F. and 420° F.

15 3. A hard bituminous material adapted for use in a storage battery compound derived from a cracked and vacuum distilled Lagunillas crude having a susceptibility factor between 27 and 35 and a softening point between 320° F. and 420° F.

20 4. A hard bituminous material adapted for use as a storage battery compound derived from a cracked and vacuum distilled mixture of Lagunillas crude and La Rosa crude having a susceptibility factor between 27 and 35 and softening point between 320° F. and 420° F.

25 5. A hard bituminous material according to claim 4 in which the mixture from which the said bituminous material is prepared is in major part Lagunillas crude and in minor part La Rosa bottoms.

30 6. A process of preparing a hard bituminous material adapted for use in a storage battery compound which comprises cracking a paraffin-free asphaltic base West Venezuela crude to a residual bottoms oil having a gravity viscosity relationship of 8° A. P. I. to 9° A. P. I. gravity and Furol viscosity of between 1000 seconds and 1400 seconds to between 600 seconds and 850 seconds at 122° F. respectively, distilling the residual oil under vacuum to obtain a residue of bituminous material having a softening point in the range between 320° F. and 420° F. and susceptibility factor of 27 to 35.

35 7. A process of preparing a hard bituminous material adapted for use as a storage battery compound which comprises cracking a paraffin-free asphaltic base Lagunillas crude to a residual bottoms oil having a gravity viscosity relationship of 8° A. P. I. to 9° A. P. I. gravity and Furol viscosity of between 1000 seconds and 1400 seconds to between 600 seconds and 850 seconds at 122° F. respectively, distilling the residual oil under vacuum to obtain a residue of bituminous material having a softening point in the range between 320° F. and 420° F. and susceptibility factor of 27 to 35.

40 8. A process of preparing a hard bituminous material adapted for use as a storage battery compound which comprises cracking a paraffin-free asphaltic base mixture of a major portion of Lagunillas crude and a minor portion of La Rosa bottoms to a residual bottom oil having a gravity viscosity relationship of 8° A. P. I. to 9° A. P. I. gravity and Furol viscosity of between 1000 seconds and 1400 seconds to between 600 seconds and 850 seconds at 122° F. respectively, distilling the residual oil under vacuum to obtain a residue of bituminous material having a softening point in the range between 320° F. and 420° F. and susceptibility factor of 27 to 35.

45 9. A process of preparing a hard bituminous material adapted for use as a storage battery compound which comprises cracking a paraffin-free asphaltic base mixture of a major portion of Lagunillas crude and a minor portion of La Rosa bottoms to a residual bottom oil having a gravity viscosity relationship of 8° A. P. I. to 9° A. P. I. gravity and Furol viscosity of between 1000 seconds and 1400 seconds to between 600 seconds and 850 seconds at 122° F. respectively, distilling the residual oil under vacuum to obtain a residue of bituminous material having a softening point in the range between 320° F. and 420° F. and susceptibility factor of 27 to 35.

softening point in the range between 320° F. and 420° F. and susceptibility factor of 27 to 35.

9. A process of preparing a hard bituminous material adapted for use in storage battery compound which comprises cracking a paraffin-free asphaltic base Lagunillas crude to a residual bottom oil having a gravity viscosity relationship of 8° A. P. I. to 9° A. P. I. gravity and Furol viscosity of between 1000 seconds and 1400 seconds to between 600 seconds and 850 seconds at 122° F. respectively, distilling the residual oil under vacuum and steam to obtain a residue of bituminous material having a softening point in the range between 320° F. and 420° F. and susceptibility factor of 27 to 35.

10. A process of preparing a hard bituminous material adapted for use in storage battery compound which comprises cracking a paraffin-free asphaltic base Lagunillas crude to a residual

bottom oil having a gravity viscosity relationship of 8° A. P. I. gravity and Furol viscosity of between 1000 seconds and 1400 seconds at 122° F., distilling the residual oil under absolute pressure 5 25 to 100 mm. with 10 to 40 lbs. of steam per barrel of charge stock to obtain a residue of bituminous material having a softening point in the range between 320° F. and 420° F. and susceptibility factor of 27 to 35.

11. A hard unoxidized bituminous material adapted for use in a storage battery compound derived from a mixture of cracked and vacuum distilled paraffin-free asphaltic base petroleum crude oils having a susceptibility factor between 15 27 and 35 and a softening point between 320° F. and 420° F. and a content of material insoluble in carbon disulfide less than 1.5%.

HENRY M. NOEL.